

1

3,364,013

### STAINLESS STEEL ALLOY

Robert L. Caton, Wyomissing, Pa., assignor to The Carpenter Steel Company, Reading, Pa., a corporation of New Jersey

No Drawing. Continuation-in-part of application Ser. No. 476,655, Aug. 2, 1965. This application Feb. 6, 1967, Ser. No. 614,029

6 Claims. (Cl. 75—126)

### ABSTRACT OF THE DISCLOSURE

Age hardenable martensitic stainless steel and article made thereof containing chromium, cobalt and molybdenum.

This application is a continuation-in-part of my application Ser. No. 476,655 filed Aug. 2, 1965, now abandoned.

This invention relates to an iron base alloy and more particularly to a chromium-cobalt-molybdenum stainless steel alloy which is age hardenable and, in that condition, is characterized by a unique combination of high strength and ductility, both at room and at elevated temperatures.

Since the advent of age hardenable martensitic iron base alloys, considerable effort has been expended toward providing a martensitic stainless steel alloy which could be readily forged, hot and/or cold worked, and which, when suitably heat treated, could be strengthened so as to provide parts having high strength and good stainless properties at temperatures ranging from room temperatures up to about 1100° F. In such alloys and that of the present application, strength is measured by tensile tests, both at room and elevated temperatures, and by stress rupture life tests at elevated temperatures. For many purposes, the usefulness of such alloys is determined to a large extent by the ultimate tensile strength of the part. For example, such parts may include structural members of steam turbine compressors or supersonic air vehicles. On the other hand, more intricately shaped parts of steam turbine compressors or the structural portions of supersonic air vehicles must not be notch sensitive, and in practice, it is usually required that the notch tensile strength of such parts be at least equal to the ultimate tensile strength.

I have discovered that by carefully balancing my composition within critically defined ranges, with particular attention to the elements chromium, cobalt and molybdenum, an age hardenable stainless steel alloy is provided which is eminently well suited for meeting the foregoing requirements. Not only does my alloy have outstanding strength, but it does not require more than a relatively simple heat treatment to convert it from the condition in which it is readily forged and hot or cold worked to a precipitation hardened martensite which combines highly desirable properties of strength, ductility and corrosion resistance. My alloy readily transforms to a martensitic structure and does not require any unusual or hard to control treatments.

The preferred and broad ranges of my composition are given in approximate weight percent in accordance with good metallurgical practice in the following table:

2

|            | Broad Range    | Preferred Range  |
|------------|----------------|------------------|
| Carbon     | 10% max        | .010% max.       |
| Manganese  | .50% max       | .10% max.        |
| Silicon    | .50% max       | .10% max.        |
| Phosphorus | .030% max      | .010% max.       |
| Sulfur     | .030% max      | .010% max.       |
| Nickel     | Up to 3.0%     | .50% max.        |
| Chromium   | 12.0% to 18.0% | 14.5% to 16.5%   |
| Cobalt     | 18.0% to 26.0% | 19.0% to 21.0%   |
| Molybdenum | 1.5% to 3.5%   | 2.0% to 3.0%     |
| Boron      | Up to .01%     | 0.001% to 0.003% |
| Iron       | Balance*       | Balance*         |

\*Except for incidental impurities.

When properly balanced within this broad range, my alloy provides an ultimate tensile strength of about 190,000 p.s.i. to 270,000 p.s.i., and a notch tensile strength, stress concentration factor of 10, of about 150,000 p.s.i. to 340,000 p.s.i. This is combined with a .2% yield strength of about 170,000 p.s.i. to 230,000 p.s.i.

20 Within the broad range, care must be exercised in balancing the composition, particularly with the larger amounts of nickel present to avoid an undesirable amount of retained austenite. Thus, with nickel in the neighborhood of 3%, I preferably use the lower amounts of the 25 alloying elements which tend to form or stabilize austenite to keep the maximum retained austenite below about 20%.

The elements cobalt and nickel are austenite formers, although nickel is much stronger in this regard, while the 30 elements chromium and molybdenum tend to form ferrite and stabilize austenite. Thus, within the broad ranges stated, these elements are balanced in my composition so that the alloys attains a stable, primarily martensitic microstructure. Substantially no retained ferrite or sigma phase is desired in my composition because those phases cause an excessive loss in ductility and embrittlement. However, larger amounts of retained austenite can be tolerated in my alloy without objectionably affecting its 35 high tensile strength, and when so balanced, is well suited for use where the outstanding stress rupture strength and notch tensile strength of my preferred composition are not required. More consistent results, particularly in the attainment of a notch tensile strength which is at least equal to or greater than the ultimate tensile strength, together with maximum yield strength and transverse ductility, are attained when my alloy is not only free of retained ferrite and sigma phase but also is essentially free of retained austenite, that is, when retained austenite is 40 less than about 5%. Within its preferred range, my alloy consistently provides parts which, in their heat treated condition, have a room temperature ultimate tensile strength of about 200,000 p.s.i. to 250,000 p.s.i., a .2% yield strength of about 180,000 p.s.i. to 225,000 p.s.i. and a notch tensile strength of about 200,000 p.s.i. to 325,000 p.s.i. Furthermore, the NTS/UTS ratio of my preferred 45 composition is consistently at least equal to or greater than one.

Carbon and nitrogen are strong austenite forming elements and advantageously are kept to a minimum in the 50 alloy. In amounts in excess of about .10%, carbon may have a beneficial effect upon the ultimate tensile strength but it excessively impairs the yield strength and results in the presence of relatively hard martensite in the as-solution-treated condition of the composition which detracts

from the formability and machineability of the alloy. Thus carbon is limited to a maximum of .10% in this alloy. However, because carbon is such a strong austenite former, care must be exercised in balancing the alloy by using the smaller amounts of the elements which form or stabilize austenite so as to ensure that the retained austenite in the alloy does not exceed 20%. When the most favorable notch tensile strength is not required, carbon may be present in this alloy in an amount of up to .10%, but balancing the alloy to ensure that the amount of retained austenite is not excessive is facilitated by limiting the carbon content to no more than .05%. Carbon appears to have its most significant objectionable effect in increasing the amount of retained austenite and in increasing the hardness of the alloy in its as-solution-treated condition when it is present in this alloy in amounts ranging from about .01% to .05%. Thus, carbon is preferably kept below .010% maximum. Nitrogen, in addition to being a strong austenite former, tends to form nitrides. It is, like carbon, therefore, considered to be an undesired impurity and is held to no more than .1%, and preferably to more than .01%.

Manganese is also a strong austenite former and is tolerated only in amounts which do not upset the martensitic balance of the alloy. When the alloy is melted in air, manganese may be used as a deoxidizer in controlled amounts so that no more than about .50% is retained in the alloy. Preferably, the amount of retained manganese is kept to no more than .10%.

Silicon may also be advantageously used as a deoxidizer when the alloy is air melted. Although silicon is a ferrite former, it too is not a desirable alloying element and is held to no more than .50% and preferably to no more than .10%.

Aluminum and titanium are commonly used strengthening agents, but in my alloy, when either or both are present in amounts of .5% or more, severe embrittlement results as indicated by a marked reduction of the notch tensile strength.

Nickel causes the formation and/or retention of undesired austenite in my alloy, and also objectionably depresses the austenite reversion temperature of the alloy with a consequent instability upon long exposure to elevated temperatures. For best results, I preferably limit nickel to no more than .50%, although I may use as much as 3% for its desirable effect upon the alloy notch tensile strength at room temperature when the accompanying loss in stress rupture strength at 1000° F. can be tolerated. With the larger amounts of nickel, the cobalt content should be adjusted downward within the stated range to preserve the martensitic balance of the alloy. The austenite stabilizing elements, e.g., chromium, can also be adjusted downward to avoid the retention of excessive austenite.

Within the limits stated, the elements chromium, cobalt, molybdenum and iron work together, and, unless these elements are carefully maintained within the specified ranges, the unique combination of properties characteristic of my alloy of high strength, together with good stainless properties, good forgeability and hot or cold workability, is not attained.

In my alloy at least about 12% chromium is required to attain the desired stainless properties, together with high ultimate and notch tensile strengths. Chromium is a ferrite forming element and also tends to stabilize austenite formed during the high temperature treatment of the alloy. This effect with the resultant retention of excess ferrite, sigma phase and/or austenite becomes increasingly apparent as the chromium content in my alloy is increased above about 18%. For best notch and ultimate tensile strengths, and to eliminate the possibility of retained ferrite, sigma phase and/or excess austenite, my alloy preferably contains from about 14.5% to 16.5% chromium.

Cobalt, like nickel, causes the formation and/or retention of austenite but has much less of an effect in this regard than nickel. Thus, as much as 26% cobalt can be used in my alloy by adjusting the austenite stabilizing elements downward within their broad ranges without its causing the retention of an undesirable amount of austenite. Below about 18% cobalt, the unique strength characteristic of my alloy is not attained. Over this range, the cobalt works with the broad ranges of chromium and molybdenum to provide my high strength stainless steel alloy, but to consistently attain high notch tensile strength so that the NTS/UTS ratio is at least equal to or greater than one and minimize retained austenite, I preferably use about 19% to 21% cobalt in my alloy. Also, the austenite stabilizing effect of chromium and cobalt is preferably offset by balancing the larger amounts of chromium with the lower amounts of cobalt, and vice versa, within the ranges already stated. Thus, with about 14.5% chromium I prefer to use about 21% cobalt, and with about 16.5% chromium I preferably balance about 19% cobalt.

Molybdenum and tungsten may be used interchangeably in my alloy. At any level of molybdenum, the amount of tungsten required to replace a given amount of molybdenum with an equivalent effect is in the proportion of about 1.2% to 1.6% tungsten to 1% molybdenum. It is therefore to be understood that throughout this application, when molybdenum is referred to, it is intended to include molybdenum and tungsten either together or individually with the tungsten replacing all or parts of the molybdenum in the proportion stated.

Molybdenum critically affects the strength of my alloy and from about 1.5% to 3.5% molybdenum (or the equivalent amount of tungsten) is essential for this purpose. The notch tensile strength of this alloy is especially sensitive to the molybdenum content. Below about 2% molybdenum, the high notch tensile strength of my preferred composition cannot be consistently attained. This is the case also when molybdenum is present in an amount greater than about 3%. Thus, to ensure consistent attainment of a NTS/UTS ratio of at least one, I preferably use from about 2% to 3% molybdenum. However, when somewhat lower notch tensile strength can be tolerated, I use the larger amounts of molybdenum to attain higher ultimate tensile and yield strengths.

When my alloy is intended for a use which requires a NTS/UTS ratio equal to or greater than one, it is balanced within the preferred range with boron ranging from about 0.001% to about 0.003%. Unless boron in this critically defined range is included when balancing the composition within the preferred range, a NTS/UTS ratio of at least equal to or greater than one cannot be consistently attained. On the other hand, when the alloy is balanced within the preferred range for a use which requires a minimum notch tensile strength of no more than about 150,000 p.s.i., then a minimum of about 0.0005% and no more than about 0.007% boron is included in the composition.

When this alloy is intended for use in the fabrication of parts or articles in which a notch tensile strength at room temperature of less than 150,000 p.s.i. can be tolerated, then boron need not be present in this alloy, or if desired, boron can be included in an amount up to about 0.01% because of its beneficial effect upon the ultimate tensile strength, the .2% yield strength and the stress rupture strength of the alloy. Furthermore, when a composition within the broader range of this alloy, but outside the preferred range, is intended for a use which requires a minimum notch tensile strength of about 150,000 p.s.i., boron may or may not be included, depending upon its effect on the notch tensile strength of the composition.

My alloy is readily prepared and formed into parts. It may be melted in air in the usual way but better results are more readily attained when the alloy is vacuum-induction melted. If desired, a double melting process may be used in which an ingot is air or vacuum-induction melted and cast, and then remelted under vacuum as a

consumable electrode. Whether the alloy is air or vacuum melted, the heat treatment required to bring out the unique properties of the alloy is relatively easy to carry out. The alloy can be solution treated from about 1400° F. to 1800° F., preferably from about 1500° F. to 1700° F., for a sufficient time to ensure complete austenitizing. Usually about one hour for each inch of thickness is sufficient. After cooling to room temperature, it is re-

Examples 1-14 had a major gauge diameter of .357 in., a notch diameter of .252 in. and a notch root radius of .001 in., a stress concentration factor ( $K_t$ ) of about 10. The results of the tests are shown in the following table and are the average of several tests, except in the case of the notch tensile strength tests where the results obtained from the individual specimens of each example are given.

TABLE II

| Ex. No. | UTS* | NTS*                     | Percent Y.S.*     | Percent Elong. | Percent R.A. | Percent Austenite |
|---------|------|--------------------------|-------------------|----------------|--------------|-------------------|
| 1       | 198  | 158<br>193<br>226        | 210<br>275<br>285 |                | 16           | 62                |
| 2       | 214  | 259<br>269<br>290<br>298 | 283<br>296        |                | 17           | 64                |
| 3       | 226  | 292<br>296               | 304<br>316        |                | 16           | 63                |
| 4       | 237  | 279<br>295               | 304               |                | 16           | 58                |
| 5       | 235  | 281<br>297               | 298<br>304        |                | 17           | 61                |
| 6       | 242  | 155<br>210<br>212<br>239 | 245<br>265        |                | 16           | 57                |
| 7       | 214  | 143<br>151<br>188        |                   | 193            | 15           | 53                |
| 8       | 249  | 279<br>295               | 300<br>303        | 220            | 16           | 59                |
| 9       | 244  | 278<br>280               | 280<br>293        | 284            | 17           | 56                |
| 10      | 235  | 280<br>288               | 306               | 309            | 15           | 59                |
| 11      | 255  | 279<br>304               | 340               | 223            | 16           | 57                |
| 12      | 254  | 199<br>251               | 258<br>304        | 225            | 17           | 55                |
| 13      | 257  | 180                      | 298               | 313            | 15           | 48                |
| 14      | 230  | 267                      | 308               | 314            | 16           | 62                |

\*1,000 p.s.i.

heated to about 900° F. to 1100° F., preferably 1000° F. to 1050° F., for about two to four hours followed by cooling in air. In the case of work pieces of substantial thickness, rapid cooling from the austenitizing temperature, as by quenching in oil or water, is used to ensure a fully transformed, martensitic microstructure.

The following specific examples of my alloy, the analyses of which, in weight percent, are set forth in Table I, as well as the examples given hereinafter for purposes of comparison, were forged into bars which were then formed into the required test specimens. The compositions were vacuum melted, and, unless otherwise noted, were heat treated for one-half hour at 1600° F. and oil quenched followed by heating for four hours at 1000° F. and then cooled in air.

TABLE I

| Ex. No. | Cr   | Co   | Mo   |
|---------|------|------|------|
| 1       | 15.0 | 20.0 | 1.55 |
| 2       | 15.0 | 19.8 | 2.10 |
| 3       | 15.0 | 19.8 | 2.46 |
| 4       | 15.0 | 20.1 | 2.86 |
| 5       | 15.0 | 20.0 | 3.02 |
| 6       | 15.0 | 20.0 | 3.22 |
| 7       | 14.0 | 20.1 | 2.97 |
| 8       | 16.1 | 19.8 | 3.00 |
| 9       | 16.8 | 19.8 | 3.01 |
| 10      | 15.2 | 20.0 | 2.93 |
| 11      | 15.2 | 21.9 | 2.93 |
| 12      | 15.1 | 22.7 | 3.05 |
| 13      | 15.1 | 23.6 | 3.05 |
| 14      | 15.1 | 19.5 | 2.94 |

In each of Examples 1-14, carbon, nitrogen, phosphorus and sulfur were each less than .01%, manganese and silicon were each less than .1%, nickel was less than .15%, boron was between 0.0005% and 0.0015%, and the remainder was iron except for incidental impurities.

Smooth bar specimens of Examples 1-14 used in carrying out measurements of ultimate tensile strength (UTS), .2% yield strength (.2% Y.S.), percent elongation (percent elong.) and percent reduction in area (percent R.A.), all of which were carried out at room temperature, had a gauge diameter of .252 in. and a gauge length of 1 in. Notch tensile strength (NTS) specimens formed of

35 In addition to the foregoing tests, elevated temperature tensile and stress rupture tests were carried out in the case of selected examples. Recorded in Table III are the results of tensile tests carried out at 1000° F. on test specimens of Examples 4 and 7-14 forged from bars prepared as was described hereinabove in connection with the room temperature test specimens but which had a gauge diameter of .357 in. and a gauge length four times the diameter.

TABLE III

| Ex. No. | .2% Y.S.* | UTS* | Percent Elong. | Percent R.A. |
|---------|-----------|------|----------------|--------------|
| 4       | 157       | 174  | 16             | 64           |
| 7       | 149       | 170  | 15             | 62           |
| 8       | 170       | 190  | 15             | 61           |
| 9       | 157       | 180  | 16             | 60           |
| 10      | 167       | 186  | 14             | 62           |
| 11      | 180       | 205  | 12             | 54           |
| 12      | 173       | 197  | 14             | 62           |
| 13      | 172       | 194  | 13             | 54           |
| 14      | 165       | 183  | 13             | 59           |

\*1,000 p.s.i.

55 Stress rupture specimens of Examples 7, 8 and 10-13 were formed from forged bars prepared as previously described and were combination notch/smooth test specimens having a smooth bar gauge diameter of .178 in. and gauge length of .712 in. The notch portion of each specimen had a notch diameter of .178 in. and major diameter of .252 in. and a notch root radius of .005 in., giving a stress concentration factor ( $K_t$ ) of about 3.8.

TABLE IV

| Ex. No. | Stress Rupture Life, hrs. <sup>1</sup> | Percent Elong. | Percent R.A. |
|---------|----------------------------------------|----------------|--------------|
| 7       | 57                                     | 20             | 64           |
| 8       | 138                                    | 17             | 56           |
| 10      | 258                                    | 17             | 54           |
| 11      | 505                                    | (2)            | (2)          |
| 12      | 358                                    | 16             | 50           |
| 13      | 208                                    | (2)            | (2)          |

<sup>1</sup> The test load was 120,000 p.s.i.<sup>2</sup> Failure occurred at the notch.

Examples 1-6 demonstrate the effect in my composition of variations in the molybdenum content. With as little as 1.55% molybdenum and with about 15% chromium, 20% cobalt and the balance essentially iron, my composition has good ultimate strength but does not provide the NTS/UTS ratio of at least one, characteristic of my preferred composition demonstrated by Examples 3, 4 and 5. It is to be noted that Example 4 is considered to be within the range of my preferred composition because the slightly higher cobalt content of 20.1% is offset by the chromium content of 15.0% being close to the lower end of the preferred chromium range. Example 6 demonstrates that high ultimate strength is attainable in my composition with molybdenum present in an amount greater than 3%, but the reliable notch tensile strength of my preferred composition as represented by a NTS/UTS ratio consistently at least equal to one is not provided.

Examples 7-10 demonstrate the effect of varying amounts of chromium with about 20% cobalt, 3% molybdenum and the balance iron. With chromium within its preferred range as in Examples 8 and 10, the exceptional notch tensile strength of my preferred composition, together with good room temperature and elevated temperature tensile properties and good stress rupture life at elevated temperatures are obtained. With a chromium content of 12%, the good tensile strength characteristic of my composition is obtained, but the stress rupture strength at elevated temperatures and the notch tensile strength at room temperature is adversely affected. Example 9 demonstrates the effect of chromium in amounts appreciably greater than 16.5% in causing the retention of in excess of 5% austenite, the maximum desired in my preferred composition.

Examples 11-14 demonstrate that my composition, within its broad range, provides highly desirable room temperature and elevated temperature tensile properties. However, as the cobalt content is increased above 21%, the outstanding notch tensile strength of my preferred composition is no longer consistently attainable and a tendency toward notch sensitivity may be noted.

The following examples demonstrate the equivalence of molybdenum and tungsten in my composition in the approximate proportion of 1 to 1.2-1.6 in weight percent. These analyses and the test specimens used in carrying out the tests recorded in Tables V-VII were prepared as previously described. In the examples of Table V, as well as all those described hereinafter, the balance of each alloy was essentially iron and other elements were held to the amounts pointed out in connection with Table I or to inconsequential amounts, unless otherwise indicated.

TABLE V

| Ex. No. | Cr   | Co   | Mo    | W    |
|---------|------|------|-------|------|
| 15..... | 15.2 | 19.5 | ..... | 1.98 |
| 16..... | 15.2 | 19.5 | ..... | 3.80 |
| 17..... | 15.2 | 19.7 | 1.99  | .99  |
| 18..... | 15.2 | 19.7 | 1.99  | 2.06 |

TABLE VI

| Ex. No. | UTS* | NTS* |     |       | Percent Elong. | Percent R.A. | Percent Austenite |
|---------|------|------|-----|-------|----------------|--------------|-------------------|
| 15..... | 197  | 270  | 190 | 187   | 15             | 61           | 5                 |
| 16..... | 239  | 282  | 293 | 325   | 17             | 63           | Nil               |
| 17..... | 224  | 293  | 280 | ..... | 16             | 62           | 4                 |
| 18..... | 242  | 257  | 195 | 282   | 17             | 60           | .....             |

\*1,000 p.s.i.

In Table VII are recorded the results of tensile tests carried out at 1000° F. on test specimens of Examples 16, 17 and 18 prepared as was described in connection with Table III.

TABLE VII

| Ex. No. | .2% Y.S.* | UTS* | Percent Elong. | Percent R.A. |
|---------|-----------|------|----------------|--------------|
| 16..... | 163       | 189  | 17             | 63           |
| 17..... | 155       | 172  | 16             | 66           |
| 18..... | 166       | 189  | 15             | 60           |

\*1,000 p.s.i.

10 Examples 19-24 were prepared to demonstrate the effect of appreciable amounts of such elements as carbon, aluminum and titanium in my composition.

TABLE VIII

| Ex. No. | Cr.   | Co    | Mo   | C     | Al    | Ti    |
|---------|-------|-------|------|-------|-------|-------|
| 19..... | 15.0  | 19.7  | 2.82 | .039  | ..... | ..... |
| 20..... | 15.0  | 19.7  | 2.82 | .048  | ..... | ..... |
| 20A*    | 14.60 | 18.45 | 2.82 | .088  | ..... | ..... |
| 21..... | 15.0  | 19.8  | 1.90 | ..... | .43   | ..... |
| 22..... | 15.0  | 19.8  | 1.90 | ..... | .92   | ..... |
| 23..... | 15.2  | 19.7  | 1.95 | ..... | ..... | .45   |
| 24..... | 15.2  | 19.7  | 1.95 | ..... | ..... | .93   |

\*Boron less than .0005%.

25 Specimens for carrying out room temperature tensile tests were prepared from each of Examples 19-24 in the same manner as was described in connection with the room temperature tensile tests described above. The results of such tests carried out on specimens of Examples 19-24 are recorded in Table IX.

TABLE IX

| Ex. No.  | UTS* | NTS*  |       |       | Percent Elong. | Percent R.A. | Percent Austenite |
|----------|------|-------|-------|-------|----------------|--------------|-------------------|
| 19.....  | 250  | 269   | 290   | 301   | 19             | 62           | 11                |
| 20.....  | 252  | 231   | 259   | 271   | 18             | 60           | 13                |
| 20A..... | 248  | 251.5 | 217.9 | 263.0 | 15.4           | 53.3         | 6                 |
| 21.....  | 205  | 90    | 122   | 139   | 13             | 54           | .....             |
| 22.....  | 211  | 121   | 127   | 140   | 8              | 33           | .....             |
| 23.....  | 58   | 71    | 77    | ..... | .....          | .....        | .....             |
| 24.....  | 228  | 81    | 81    | 83    | 10             | 37           | .....             |

\*1,000 p.s.i.

45 Examples 19, 20 and 20A demonstrate the effect of the larger amounts of carbon upon the retention of austenite and the notch tensile strength of my alloy. In Example 20A the effect of carbon on the retention of austenite is counter-acted by the reduction in the chromium and cobalt contents as compared to Examples 19 and 20. Examples 21-24 demonstrate that appreciable amounts of aluminum and titanium severely reduce the ductility and notch tensile strength of my alloy.

50 Examples 25, 26 and 27 were prepared to demonstrate the effect of nickel in my composition and the analyses and test data are set forth in Table X.

55

TABLE X

| Elements and Tests                                       | Ex. 25        | Ex. 26        | Ex. 27        |
|----------------------------------------------------------|---------------|---------------|---------------|
| Cr.....                                                  | 15.3          | 15.2          | 15.3          |
| Co.....                                                  | 19.9          | 15.1          | 19.9          |
| Mo.....                                                  | 2.86          | 2.86          | 2.86          |
| Ni.....                                                  | 1.00          | 3.03          | 2.93          |
| Room Temp., Tensile Data:                                |               |               |               |
| UTS*.....                                                | 244           | 222           | 139           |
| NTS*.....                                                | 327, 334, 336 | 331, 326, 331 | 149, 150, 166 |
| Percent Elong.....                                       | 17            | 17            | 38            |
| Percent R.A.....                                         | 61            | 63            | 72            |
| Percent Austenite.....                                   | 10            | 13            | 75            |
| 1,000° F., Tensile Data:                                 |               |               |               |
| .2% Y.S.....                                             | 163           | 147           | .....         |
| UTS*.....                                                | 185           | 163           | .....         |
| Percent Elong.....                                       | 14            | 14            | .....         |
| Percent R.A.....                                         | 58            | 61            | .....         |
| 1,000° F., 120,000 p.s.i., Stress Rupture Life, hrs..... | 71            | 7             | .....         |
| Percent Elong.....                                       | 21            | 19            | .....         |
| Percent R.A.....                                         | 54            | 60            | .....         |

75 \*1,000 p.s.i.

With only 1% nickel, the adverse effect upon the stress rupture life of my composition at elevated temperatures is apparent from Example 25, but it will be noted that Example 25 and Example 26 demonstrate highly desirable room temperature properties. Example 26 further demonstrates the severe effect of 3% nickel upon the elevated temperature stress rupture life of my composition and that it is not compensated for even when the cobalt content is reduced below the minimum of 18% to as low as 15.1%. When the consequent impairment of elevated temperature stress rupture life can be tolerated, I may use as much as 3% nickel, but in that event, the other elements which form or stabilize austenite are held to the lower amounts hereinbefore indicated in order to maintain the essentially martensitic balance of the composition with preferably no more than about 20% retained austenite. Example 27 demonstrates that unless the balance of the alloy is adjusted by reducing the cobalt content to avoid the retention of excessive amounts of austenite, the room temperature tensile properties are severely affected by an addition of 2.93% nickel.

In my composition, the elements chromium, cobalt and molybdenum must be carefully maintained within the ranges stated. When any one of those elements is present either in an amount appreciably below or above the broad range stated for that element, then the tensile properties or strength characteristic of my alloy is not attained. Referring to Table XI, Examples 28 and 29 demonstrate the severe effect of excessive amounts of molybdenum and/or tungsten upon the notch tensile strength of the alloy. With 4.03% and 3.90% molybdenum in those respective examples, there is a marked loss in notch tensile strength, although an ultimate tensile strength of about 250,000 p.s.i. is attained.

TABLE XI

| Elements and Tests            | Ex. 28 | Ex. 29 | Ex. 30 | Ex. 31 | Ex. 32 | Ex. 33 |
|-------------------------------|--------|--------|--------|--------|--------|--------|
| Cr.....                       | 15.0   | 15.2   | 13.0   | 18.2   | 15.0   | 14.9   |
| Co.....                       | 19.9   | 20.1   | 19.8   | 19.8   | 16.0   | 25.6   |
| Mo.....                       | 4.03   | 3.90   | 3.03   | 3.00   | 2.95   | 3.10   |
| Room Temp., Tensile Data:     |        |        |        |        |        |        |
| UTS <sup>1</sup> .....        | 253    | 255    | 206    | 159    | 198    | 207    |
| NTS <sup>1</sup> .....        | 100    | 139    | 195    | 135    | 155    | 211    |
| 105                           | 178    | 160    | 146    | 192    | 209    |        |
| 125                           | 181    | 200    | 155    | 155    | 125    |        |
| 140                           |        |        | 112    |        |        |        |
| 130                           |        |        |        |        |        |        |
| 151                           |        |        |        |        |        |        |
| .2% Y.S.....                  |        |        | 182    | 113    |        |        |
| Percent Elong.....            | 13     | 15     | 20     | 17     | 15     |        |
| Percent R.A.....              | 51     | 55     | 62     | 62     | 62     |        |
| Percent Austenite.....        | Nil    | 5      | Nil    | 57     | Nil    | 33     |
| 1,000° F., Tensile Data:      |        |        |        |        |        |        |
| .2% Y.S. <sup>1</sup> .....   | 181    | 142    | 91     | 140    | 96     |        |
| UTS <sup>1</sup> .....        | 210    | 167    | 115    | 156    | 129    |        |
| Percent Elong.....            | 14     | 14     | 16     | 16     | 17     |        |
| Percent R.A.....              | 66     | 64     | 42     | 65     | 52     |        |
| 1,000° F., 120,000 p.s.i.:    |        |        |        |        |        |        |
| Stress Rupture Life, hrs..... |        | 24     | 81     |        |        |        |
| Percent Elong.....            |        | 30     | 19     |        |        |        |
| Percent R.A.....              |        | 53     | 60     |        |        |        |

<sup>1</sup> 1,000 p.s.i.<sup>2</sup> 100,000 p.s.i.

Example 30 demonstrates the effect of less than my preferred amounts of chromium upon notch tensile strength, but this analysis is suitable for use where an NTS/UTS ratio greater than 1 is not required. Example 31 is essentially the same as Example 30 but for the chromium content of 18.2%. The test data clearly demonstrates the loss in strength and the excessive amount of retained austenite. Example 32 demonstrates the effect of an insufficient amount of cobalt while Example 33 demonstrates the need for care in balancing the alloy when the larger amounts of cobalt within the broad range are used. Better over-all properties are attained when, with as much as 25.6% cobalt, the chromium content is reduced somewhat. Also the molybdenum content may be reduced to the neighborhood of about 2% with such a larger amount of cobalt present.

The outstanding properties of my alloy are readily obtained when it is prepared in commercial quantities so as to contain 14.8% to 15.5% chromium, 19.75% to 20.25% cobalt, 2.75% to 3.00% molybdenum, and the remaining elements as stated in connection with the preferred range set forth hereinabove. For example a 2500 pound ingot was vacuum induction melted and then remelted as a consumable electrode under vacuum. The final ingot thus formed had the following analysis, in weight percent:

|                     | Percent                                  |
|---------------------|------------------------------------------|
| Carbon .....        | 0.008                                    |
| Manganese .....     | 0.08                                     |
| Silicon .....       | 0.06                                     |
| 15 Phosphorus ..... | 0.007                                    |
| Sulfur .....        | 0.005                                    |
| Nickel .....        | 0.22                                     |
| Chromium .....      | 15.00                                    |
| Cobalt .....        | 20.16                                    |
| 20 Molybdenum ..... | 2.97                                     |
| Boron .....         | 0.001                                    |
| Iron .....          | Balance except for incidental impurities |

The ingot was heated to its hot working range, 1900-2100° F. and was readily hot worked to form various products including billets, bars, strip and wire. Examination of the microstructure of specimens of the various products showed that they contained less than 5% retained austenite with no detectable retained ferrite or sigma phase. Test specimens were formed as was described in connection with Examples 1-14, the heat treatment of which consisted of heating to 1700° F. for one-half hour followed by oil quenching and then aging at 1025° F. for four hours followed by cooling in air.

At room temperature the .2% yield strength was from 220,000 p.s.i.-22,000 p.s.i. The ultimate tensile strength was from 240,000 to 245,000 p.s.i., with about 18% elongation and 60% reduction in area. The notch tensile strength was from 280,000 to 330,000 p.s.i. The alloy as solution treated was found to have a hardness of Rockwell C 30, and as aged, a hardness of Rockwell C 49.

At 1000° F. the .2% yield strength was 175,000 p.s.i. and the ultimate tensile strength was 190,000 p.s.i. with 16% elongation and 60% reduction in area. The stress rupture life at 1000° F. under a load of 125,000 p.s.i. was measured on specimens formed both from billets and from bar stock. One test specimen formed from a billet withstood the load of 125,000 p.s.i. for a 133 hour period and showed an elongation of 26% and a reduction in area of 64%. A second specimen withstood the load for 165 hours and showed an 18% elongation and a 56% reduction in area. A third specimen withstood the load of 125,000 p.s.i. for 121 hours and showed a 25% elongation and 65% reduction in area. One test specimen formed from bar stock withstood the load of 125,000 p.s.i. for 175 hours with 21% elongation and 59% reduction in area.

The terms and expressions which have been employed are used as terms of description and not of limitation, and there is no intention, in the use of such terms and expressions, of excluding any equivalents of the features described or portions thereof, but it is recognized that various modifications are possible within the scope of the invention claimed.

What is claimed is:

1. An age hardenable stainless iron base alloy which in its age hardened condition is characterized by an ultimate tensile strength of above about 190,000 p.s.i. with good ductility and which consists essentially of by weight a maximum of 0.10% carbon, a maximum of 0.50% manganese, a maximum of 0.50% silicon, a maximum of 0.030% phosphorus, a maximum of 0.030% sulfur, no more than about 3% nickel, from about 12% to 18% chromium, from about 18% to 26% cobalt, from about 1.5% to 3.5% molybdenum or an equivalent amount of tungsten with tungsten replacing molybdenum in the ratio 75 of about 1.2% to 1.6% tungsten to 1% molybdenum, up

to about 0.01% boron, the remainder being substantially iron, and said alloy being balanced so as to have a primarily martensitic microstructure substantially free of retained ferrite and sigma phase following heat treatment and aging at elevated temperatures.

2. An age hardenable stainless iron base alloy which in its age hardened condition is characterized by an ultimate tensile strength of at least about 200,000 p.s.i. with good ductility and with a ratio of notch tensile strength to ultimate tensile strength at least equal to or greater than one at a stress concentration factor of 10 and which consists essentially of by weight a maximum of 0.010% carbon, a maximum of 0.10% manganese, a maximum of 0.10% silicon, a maximum of 0.010% phosphorus, a maximum of 0.010% sulfur, no more than about 0.50% nickel, from about 14.5% to 16.5% chromium, from about 19.0% to 21.0% cobalt, from about 2.0% to 3.0% molybdenum or an equivalent amount of tungsten with tungsten replacing molybdenum in the ratio of about 1.2% to 1.6% tungsten to 1% molybdenum, from about 0.001% to 0.003% boron, the remainder being substantially iron, and said alloy following heat treatment and aging at elevated temperatures having an essentially martensitic microstructure substantially free of retained ferrite and sigma phase and containing no more than about 5% retained austenite.

3. A stainless steel article formed from an alloy which consists essentially of by weight a maximum of 0.10% carbon, a maximum of 0.50% manganese, a maximum of 0.50% silicon, a maximum of 0.030% phosphorus, a maximum of 0.030% sulfur, no more than about 3% nickel, from about 12% to 18% chromium, from about 18% to 26% cobalt, from about 1.5% to 3.5% molybdenum or an equivalent amount of tungsten with tungsten replacing molybdenum in the ratio of about 1.2% to 1.6% tungsten to 1% molybdenum, up to about 0.01% boron, the remainder being substantially iron, the composition of said article being balanced and the article being heat treated and age hardened at elevated temperatures to have a primarily martensitic microstructure substantially free of retained ferrite and sigma phase with an ultimate tensile strength of above about 190,000 p.s.i., good ductility, a notch tensile strength of above about 150,000 p.s.i. at a stress concentration factor of 10 and with a .2% yield strength of above about 170,000 p.s.i.

4. A stainless steel article formed from an alloy which consists essentially of by weight a maximum of 0.010% carbon, a maximum of 0.10% manganese, a maximum of 0.10% silicon, a maximum of 0.010% phosphorus, a maximum of 0.010% sulfur, no more than about 0.50% nickel, from about 14.5% to 16.5% chromium, from about 19.0% to 21.0% cobalt, from about 2.0% to 3.0% molybdenum or an equivalent amount of tungsten with tungsten replacing molybdenum in the ratio of about 1.2% to 1.6% tungsten to 1% molybdenum, from about 0.001% to 0.003% boron, the remainder being substantially iron, said article being heat treated and age hardened at elevated temperatures and having an ultimate tensile strength of above about 200,000 p.s.i. with good ductility and with a ratio of notch tensile strength to ultimate tensile strength at least equal to or greater than one at a stress concentra-

tion factor of 10 and a .2% yield strength of above about 180,000 p.s.i. and said article having an essentially martensitic microstructure substantially free of retained ferrite and sigma phase and containing no more than about 5% retained austenite.

5. An age hardenable stainless iron base alloy which in its age hardened condition is characterized by an ultimate tensile strength of at least about 200,000 p.s.i. with good ductility and with a ratio of notch tensile strength to ultimate tensile strength at least equal to or greater than one at a stress concentration factor of 10 and which consists essentially of by weight a maximum of 0.010% carbon, a maximum of 0.10% manganese, a maximum of 0.10% silicon, a maximum of 0.010% phosphorus, a maximum of 0.010% sulfur, no more than about 0.50% nickel, from about 14.8% to 15.5% chromium, from about 19.75% to 20.25% cobalt, from about 2.75% to 3.0% molybdenum or an equivalent amount of tungsten with tungsten replacing molybdenum in the ratio of about 1.2% to 1.6% tungsten to 1% molybdenum, from about 0.001% to 0.003% boron, the remainder being substantially iron, and said alloy following heat treatment and aging at elevated temperatures having an essentially martensitic microstructure substantially free of retained ferrite and sigma phase and containing no more than about 5% retained austenite.
6. A stainless steel article formed from an alloy which consists essentially of by weight a maximum of 0.010% carbon, a maximum of 0.10% manganese, a maximum of 0.10% silicon, a maximum of 0.010% phosphorus, a maximum of 0.010% sulfur, no more than about 0.50% nickel, from about 14.8% to 15.5% chromium, from about 19.75% to 20.25% cobalt, from about 2.75% to 3.0% molybdenum or an equivalent amount of tungsten with tungsten replacing molybdenum in the ratio of about 1.2% to 1.6% tungsten to 1% molybdenum, from about 0.001% to 0.003% boron, the remainder being substantially iron, said article being heat treated and age hardened at elevated temperatures and having an ultimate tensile strength of above about 200,000 p.s.i. with good ductility and with a ratio of notch tensile strength to ultimate tensile strength at least equal to or greater than one at a stress concentration factor of 10 and a .2% yield strength of above about 180,000 p.s.i., and said article having an essentially martensitic microstructure substantially free of retained ferrite and sigma phase and containing no more than about 5% retained austenite.

#### References Cited

##### UNITED STATES PATENTS

|    |           |         |         |       |          |
|----|-----------|---------|---------|-------|----------|
| 50 | 2,848,323 | 8/1958  | Harris  | ----- | 75—126 X |
|    | 2,880,085 | 3/1959  | Kirkby  | ----- | 75—126   |
|    | 2,985,529 | 5/1961  | Harris  | ----- | 75—126   |
|    | 2,990,275 | 6/1961  | Binder  | ----- | 75—126   |
| 55 | 3,154,412 | 10/1964 | Basak   | ----- | 75—126   |
|    | 3,251,683 | 5/1966  | Hammond | ----- | 75—128   |

DAVID L. RECK, Primary Examiner.

P. WEINSTEIN, Assistant Examiner.

UNITED STATES PATENT OFFICE  
CERTIFICATE OF CORRECTION

Patent No. 3,364,013

January 16, 1968

Robert L. Caton

It is hereby certified that error appears in the above numbered patent requiring correction and that the said Letters Patent should read as corrected below.

In the heading to the printed specification, line 3, for "Wyomissing" read -- Wyomissing Hills --; column 2, line 33, for "alloys" read -- alloy --; line 54, for "325,000" read -- 300,000 --; column 3, line 22, for "to more" read -- to no more --; column 4, line 28, for "parts" read -- part --; column 5, line 72, for "elong." read -- Elong. --; column 10, line 36, for "22,000" read -- 225,000 --; column 12, line 55, for "Basak" read -- Kasak --.

Signed and sealed this 1st day of April 1969.

(SEAL)

Attest:

Edward M. Fletcher, Jr.

Attesting Officer

EDWARD J. BRENNER

Commissioner of Patents